

1

3,182,020  
STABILIZED CALCIUM ACETATE OIL  
DISPERSIONS

Robert H. Davis, Woodbury, N.J., assignor to Socony 5  
Mobil Oil Company, Inc., a corporation of New York  
No Drawing. Filed June 30, 1961, Ser. No. 120,938  
5 Claims. (Cl. 252—40.7)

The invention relates to lubricating compositions. 10 More particularly it is concerned with the provision of stable dispersions of calcium acetate in lubricating oil, which dispersions are highly advantageous for use as lubricants per se or as components for lubricant compositions, including fluid lubricating oils and greases.

It is known that calcium acetate when dispersed in a lubricating oil imparts desirable improvements thereto, such as load-carrying ability and anti-wear properties. Also, because of its acid-neutralizing ability calcium acetate is a particularly desirable additive for lubricating oils used in engines operated on high sulfur-content fuels, such as marine diesel engines.

Simple dispersions of calcium acetate in lubricating oil, however, are unstable, the calcium acetate separating out during transportation and/or storage of the oil composition. In order to overcome this problem and obtain insofar as possible the advantages provided by calcium acetate, particularly in fluid lubricants such as marine diesel oils, it has been the practice to employ emulsion type oils, i.e., those formed by emulsifying a water solution of calcium acetate with lubricating oil. These emulsion oils, however, have not been entirely satisfactory. Thus, due to their water contents, they tend to increase the corrosion problem and they are unstable under the varying conditions encountered in storage and use. For example, the high temperatures encountered during storage in the engine rooms of ships tend to break the emulsion. On the other hand, under the low temperature conditions often encountered in cold climates, the aqueous phase can become frozen so that the emulsion is destroyed.

It will be appreciated that a means for providing a stable dispersion of calcium acetate in lubricating oil would be of considerable value to the art since such a "single-phase" oil will avoid the afore-mentioned disadvantages of the emulsion type oil. Furthermore, the single-phase oil will, of course, have a much wider application than emulsion type oils, such as use as a crankcase oil in spark-ignition engines and regular (non-marine) diesel engines. Such a means is provided by the present invention.

It has now been found in accordance with this invention that oil dispersions of calcium acetate, which are not only highly stable but which have a number of other unexpected and outstanding properties as lubricants and lubricant additives, can be prepared by the use therein in conjunction with the calcium acetate of small amounts of certain N-acyl-substituted sarcosine compounds. Thus, it has been found that the N-acyl-substituted sarcosine-calcium acetate dispersions prepared in accordance with this invention are not only highly stable, but are excellent viscosity index improving additives for mineral lubricating oils.

It has also been found in accordance with this invention that the consistency of the dispersions provided herein can be varied according to the end use desired, i.e., they may range from fluid oils to greases, depending upon the proportions of calcium acetate and N-acyl sarcosine utilized in their preparation. Surprisingly, it has been found that the grease dispersions are formed even with small proportions of calcium acetate which, in the absence of the sarcosine compound, will not provide a grease.

2

Accordingly, it is an object of this invention to provide novel, stabilized dispersions of calcium acetate in lubricating oil. It is another object to provide lubricant compositions comprising such dispersions, which compositions exhibit unexpected advantageous properties. Other and further objects will be apparent from the following detailed description of the invention.

The N-acyl-substituted sarcosines which are utilized as stabilizers for the calcium acetate oil dispersions in accordance with the invention conform to the formula:



15 wherein R represents an aliphatic hydrocarbon radical having from about 8 to about 24 carbon atoms and which may be either saturated or unsaturated. Typical examples of these sarcosines are the following:

20 N-pelargonoyl sarcosine  
N-undecyloyl sarcosine  
N-lauroyl sarcosine  
N-myristoyl sarcosine  
N-palmitoyl sarcosine  
25 N-stearoyl sarcosine  
N-oleoyl sarcosine  
N-linoleoyl sarcosine  
N-arachidoyl sarcosine  
N-behenoyl sarcosine  
30 N-hyеноyl sarcosine

A number of the N-acyl-substituted sarcosines are available commercially under the tradename "Sarkosyl," for example, "Sarkosyl-L" (lauroyl sarcosine), "Sarkosyl-O" (oleoyl sarcosine) and "Sarkosyl-S" (stearoyl sarcosine).

35 Either anhydrous or hydrated calcium acetate may be used in forming the dispersions of the invention. The calcium acetate may either be preformed or it may be formed in situ. When using preformed calcium acetate, the dispersion is prepared by forming a mixture of the acetate, the N-acyl-sarcosine and the base oil and stirring the mixture for a short period, say, from a few seconds up to about 30 minutes at a temperature of from about 25° C. to about 200° C. and preferably from about 50° C. to about 150° C. Although, as brought out herein-after, stable dispersions can be formed at room temperature with only a brief initial mixing of the calcium acetate, the sarcosine compound and the oil and allowing the mixture to stand for several hours, its formation is considerably hastened by heating and stirring the mixture.

40 45 50 Also, if desired, the mixture may be subjected to a mechanical homogenization treatment although this step is not essential.

The calcium acetate may be prepared in situ by neutralizing calcium oxide or calcium hydroxide with either 55 acetic anhydride or acetic acid in the presence of the oil and then heating the mixture to a temperature sufficient to remove any free water therefrom, i.e., above 100° C. The N-acyl-sarcosine is then added and the dispersion formed as in the case of the preformed calcium acetate.

60 A full understanding of the invention will be had from the following examples and tests illustrating the principles and advantages thereof.

The base oils used in the examples were as follows:

65 Base Oil No. 1—An oil typical of those used in the formulation of gear oils composed of 82%, by weight, of 125 SUS at 210° F. solvent-refined bright stock and 18%, by weight, of 200 SUS at 100° F. solvent-refined neutral oil.

70 Base Oil No. 2—An oil typical of those used in the formulation of marine diesel cylinder oils, i.e., a 60 SUS at 210° F. solvent-refined coastal stock.

Base Oil No. 3—An oil typical of those used in compounding cross-graded motor oil, i.e., a 130 SUS at 100° F. solvent-refined paraffin oil.

Base Oil No. 4—An oil typical of stocks used in metal processing oils, i.e., a 100 SUS at 100° F. solvent-refined paraffin oil.

#### EXAMPLE 1

| Materials used:                                                                     | Amount (parts by weight) |
|-------------------------------------------------------------------------------------|--------------------------|
| Calcium acetate (ctg. 6% water, i.e., approx. $\frac{2}{3}$ mol water of hydration) | 10                       |
| Oleoyl sarcosine                                                                    | 0.5                      |
| Base Oil No. 1                                                                      | 89.5                     |

*Procedure.*—To a slurry of the calcium acetate in approximately  $\frac{1}{3}$  of the base oil the sarcosine was added and the mixture stirred and heated over a period of  $\frac{1}{2}$  hour to a final temperature of about 135° C. The remainder of the base oil was then added and the mixture cooled to about 80° C. and passed through a Manton-Gaulin homogenizer operating at 3000 p.s.i. The resulting dispersion had excellent fluidity and exhibited only a slight haze.

#### EXAMPLE 2

A second dispersion was prepared after the fashion of Example 1, except that in this case 20 parts of calcium acetate,  $1\frac{1}{2}$  parts of oleoyl sarcosine and 78.5 parts of Base Oil No. 2 was used. Also, homogenization was omitted. The resulting dispersion was a viscous fluid and had only a very slight haze.

#### EXAMPLE 3

A dispersion was prepared after the fashion of Example 1, but using 40 parts of calcium acetate, 3 parts of oleoyl sarcosine and 57 parts of Base Oil No. 2. Also, all of the oil was used initially. The resulting dispersion was a smooth light colored grease.

#### EXAMPLE 4

Another dispersion was prepared after the fashion of Example 1, but in this case along with the 10 parts of calcium acetate, 2.5 parts of oleoyl sarcosine and 87.5 parts of Base Oil No. 2 were used. Also, homogenization was omitted. In this case the resulting dispersion was a smooth, light-colored grease.

#### EXAMPLE 5

A dispersion was prepared after the fashion of Example 1, utilizing the 10 parts of calcium acetate, but in this case 1 part of stearoyl sarcosine and 89 parts of Base Oil No. 4 were used and the homogenization step omitted. The dispersion obtained was a thixotropic fluid and had a moderate haze.

#### EXAMPLE 6

A preparation was carried out after the fashion of Example 5 except that here the stabilizer used was lauroyl sarcosine. The dispersion again was a thixotropic fluid with a moderate haze.

It will be seen that the dispersions of the examples varied in consistency from fluids to greases. Also, it is seen that Example 1, which was fluid, and Example 4, which was a grease, contained the same concentration (10%) of calcium acetate but different amounts of oleoyl sarcosine, Example 1 containing only 0.5% and Example 4 containing 2.5%. Accordingly, it is seen that varying the amounts of either the calcium acetate or the stabilizer or both, the consistency of the product dispersion can be controlled according to the end use desired.

The dispersions of all of the foregoing examples were stored at room temperature for a period of 3 months. During this time none of them exhibited any change in clarity, consistency or homogeneity thereby manifesting their excellent stability.

It will be seen that in the previous examples, the ratio of calcium acetate to oleoyl sarcosine varied from 20:1 (Example 1) down to 4:1 (Example 4). In Examples 7 to 10 which follow, the proportion of calcium acetate was further decreased providing ratios of calcium acetate to oleoyl sarcosine of from 1:1 to 1:8. In these examples anhydrous calcium acetate was used. The dispersions were prepared by mixing the calcium acetate, the sarcosine compound and the oil and heating the mixture with stirring to 150° C. in the course of 20 to 30 minutes at which point the heating was stopped and the mixture allowed to cool with stirring to about 90° C. The stirring was then stopped and the material allowed to reach room temperature. The data with respect to these dispersions is summarized in Table I.

It will be noted from Table I that here again, as with Examples 1 to 6, the consistency of the several dispersions varied with the ratio of calcium acetate to oleoyl sarcosine used.

To demonstrate the effectiveness of the dispersions of the invention in improving the viscosity index of lubricating oil, the dispersions of Examples 7 to 10 were cut back with additional amounts of the same mineral oil (Base Oil No. 3). In general, 2%, by weight, of the respective "concentrates" were diluted with 98%, by weight, of the oil. The amounts of total additive in the finished blends (Examples 11 to 15) are shown in Table II, together with the viscosity indices of the finished blends.

As will be seen from Table II, the dispersions of the invention are highly effective viscosity index improvers, provided a proper acetate:sarcosine ratio is selected. For instance, Example 11, using a 1:1 ratio of acetate to sarcosine raises the viscosity index of the base oil from 105 to 143, an improvement of 38 points. A similar improvement (37 points) is afforded by a 1:4 ratio (Example 13). Example 12 represents the optimum inasmuch as it provides an improvement in viscosity index of 47 points over the base oil. On the other hand, an acetate:sarcosine ratio of 1:8 (Example 14) fails to improve the viscosity index when using an equivalent acetate concentration and this lack of effectiveness is not greatly altered when the concentration is increased five-fold (Example 15).

Table I

| Ex. No. | Calcium acetate (weight percent) | Oleoyl sarcosine (weight percent) | Base Oil No. 3 (weight percent) | Consistency         | Clarity       | Stability, 3 months at rm. temp. |
|---------|----------------------------------|-----------------------------------|---------------------------------|---------------------|---------------|----------------------------------|
| 7-----  | 2.5                              | 2.5                               | 95.0                            | Viscous semi-solid. | Slight haze.. | Stable.                          |
| 8-----  | 2.5                              | 5.0                               | 92.5                            | do.....             | do.....       | Do.                              |
| 9-----  | 2.5                              | 10                                | 87.5                            | do.....             | do.....       | Do.                              |
| 10----- | 2.5                              | 20                                | 77.5                            | Fluid.....          | do.....       | Do.                              |

Table II

| Example Number | Composition of blend (weight percent) | Acetate: sarcosine ratio | Cone. of active materials (weight percent) | Viscosity index |
|----------------|---------------------------------------|--------------------------|--------------------------------------------|-----------------|
| 11.            | 100% mineral oil                      |                          | 0                                          | 105             |
| 11.            | 2% example 7, 98% mineral oil         | 1:1                      | 0.1                                        | 143             |
| 12.            | 2% example 8, 98% mineral oil         | 1:2                      | 0.15                                       | 152             |
| 13.            | 2% example 9, 98% mineral oil         | 1:4                      | 0.25                                       | 142             |
| 14.            | 2% example 10, 98% mineral oil        | 1:8                      | 0.45                                       | 105             |
| 15.            | 10% example 10, 90% mineral oil       | 1:8                      | 2.25                                       | 110             |

It is seen that the rather marked improvements in viscosity index are brought about by rather low concentrations of the active ingredients, i.e., only 0.05% of the acetate and sarcosine compound, respectively (Example 11). On this basis, significant improvements would be expected at concentrations as low as 0.01% of each material. On the other hand, concentrations above 0.05% of calcium acetate should not adversely affect the viscosity index improvement obtained, provided the proper ratio of acetate to sarcosine (1 part acetate to from 1 up to about 4 parts of sarcosine) is used.

A further unexpected advantage of the present invention is the substantial simplification of the process for preparing calcium acetate dispersions permitted by the use of the N-acyl-substituted sarcosine stabilizer. Thus, it has been found that stable dispersions of the calcium acetate can be formed with only the briefest mixing of the acetate, the oil and the stabilizer at room temperature. Thus, by simply bringing these materials together and stirring for not more than a few seconds, say, from 5 to 30 seconds, and then allowing the mixture to stand, a homogeneous dispersion forms in a short time, i.e., from about 1 to about 2 hours. This is illustrated by the following example.

#### EXAMPLE 16

Ten parts, by weight, of calcium acetate containing approximately  $\frac{1}{2}$  mol of water of hydration, 2.5 parts of oleoyl sarcosine and 40 parts of Base Oil No. 3 were stirred together at room temperature for 15 seconds. The mixture was then allowed to stand at room temperature and was examined periodically with the following results.

| Elapsed time: | Observations on mixture                                |
|---------------|--------------------------------------------------------|
| Initial       | Turbid - containing particles of crystalline material. |
| 2 hours       | Homogeneous, faintly turbid, semi-fluid dispersion.    |
| 2 weeks       | No change.                                             |

It is seen from the foregoing that a stabilized homogeneous dispersion can be prepared without significant agitation, without application of heat and without mechanical homogenization, thus providing a distinct economic advantage in the preparation of calcium acetate dispersions.

It will be appreciated that the dispersions of the invention may be used per se as lubricants, or they may be blended with base oils to provide enhanced properties therein, such as load-carrying ability, anti-wear properties, enhanced viscosity index characteristics, etc. In general, therefore, the dispersions may contain from about 0.01% to about 50% of calcium acetate and from about 0.01% to about 20% of the sarcosine compound, the amounts and the proportion of calcium acetate and sarcosine utilized in any one instance depending upon the end use for which the particular dispersion is intended. Also, the dispersions may be utilized in lubricant compositions containing other additives designed to provide various improving effects therein, such as detergents, antioxidants, pour point depressants, defoamants, etc.

Although the present invention has been described herein in terms of specific embodiments and examples thereof, it is not intended that the scope thereof be limited

in any way thereby, but only as indicated in the following claims.

What is claimed is:

1. A lubricating composition comprising a base lubricant selected from the group consisting of lubricating oils and greases having dispersed therein up to about 50%, based on the weight of the total composition, of calcium acetate and an amount sufficient to maintain said calcium acetate in a dispersed state of an N-acyl-substituted sarcosine compound of the formula



where R represents an aliphatic hydrocarbon radical of from about 8 to about 24 carbon atoms.

2. A lubricating composition comprising a lubricating oil having dispersed therein from about 0.01% to about 50%, based on the weight of the total composition, of calcium acetate and as a dispersion stabilizer from about 0.01% to about 20%, based on the weight of the total composition, of an N-acyl-substituted sarcosine compound of the formula



where R represents an aliphatic hydrocarbon radical of from about 8 to about 24 carbon atoms.

3. A lubricating composition comprising a lubricating oil having dispersed therein from about 0.01% to about 50%, based on the weight of the total composition, of calcium acetate and as a dispersion stabilizer from about 0.01% to about 20%, based on the weight of the total composition, of oleoyl sarcosine.

4. A lubricating composition comprising a lubricating oil having dispersed therein from about 0.01% to about 50%, based on the weight of the total composition, of calcium acetate and as a dispersion stabilizer from about 0.01% to about 20%, based on the weight of the total composition, of stearoyl sarcosine.

5. A lubricating composition comprising a lubricating oil having dispersed therein from about 0.01% to about 50%, based on the weight of the total composition, of calcium acetate and as a dispersion stabilizer from about 0.01% to about 20%, based on the weight of the total composition, of lauroyl sarcosine.

#### References Cited by the Examiner

#### UNITED STATES PATENTS

|           |      |                      |          |
|-----------|------|----------------------|----------|
| 2,790,779 | 4/57 | Spivack et al. ----- | 252-51.5 |
| 2,841,555 | 1/58 | Lyons et al. -----   | 252-33.6 |
| 2,940,932 | 6/60 | Morway -----         | 252-40.5 |
| 2,927,892 | 3/60 | Morway -----         | 252-39   |
| 2,929,783 | 3/60 | Morway -----         | 252-40.5 |

(Other references on following page)

## OTHER REFERENCES

Schwartz et al.: "Surface Active Agents," Interscience Publishers, Inc., New York 1949, pp. 34-55 relied on.

J. Soc. Cosm. Chem., vol. 6, No. 5, December 1955, pages 407-415, Sussman et al., "Acylated Amino Acids in Shampoos."

"Geigy Surfactants," Geigy Chemical Corporation, New York, pp. 1 and 2 relied on. (Copyright 1959.)

DANIEL E. WYMAN, *Primary Examiner.*

5 JOSÉPH R. LIBERMAN, ALPHONSO D. SULLIVAN,  
*Examiners.*